

Oct. 31, 1950

B. E. ROETHELI

**2,527,575**

## METHOD FOR HANDLING FUELS

Filed Dec. 4, 1945

2 Sheets-Sheet 1



Bruno E. Roetheli Inventor

By Ph. Young Attorney

Oct. 31, 1950

B. E. ROETHELI

**2,527,575**

## METHOD FOR HANDLING FUELS

Filed Dec. 4, 1945

2 Sheets-Sheet 2



Bruno E. Roetheli Inventor

By P. H. Young Attorney



tinuously withdrawn and the coke is subjected in a second reaction zone to a gasification reaction producing valuable fuel gases and proceeding at a temperature substantially higher than that of the coking zone. Fuel gases are recovered from said second zone and solid gasification residue is preferably continuously returned at or at about the gasification temperature to the coking zone in amounts sufficient to supply at least a substantial part of the heat required for coking.

Steam, inert gas, water gas, natural gas, flue gases or the like may be used to fluidize the solids in the coking zone which may be maintained at temperatures varying from 800° to about 1200° F. If desired, a portion of the heat required in the coking zone may be supplied by partial combustion within the coking zone. An oxidizing gas, such as air or oxygen or mixtures thereof, may replace part or all of the fluidizing gas for this purpose.

The gasification zone may be operated to produce water gas, producer gas, mixtures of carbon monoxide and hydrogen suitable for the catalytic synthesis of liquid hydrocarbons or fuel gases rich in carbon monoxide or the like at temperatures falling within the approximate range of 1200° to 2500° F. For the production of water gas or synthesis gas, steam and sufficient oxygen to support the combustion needed for the heat balance requirements in the gasification and coking zones are supplied preferably simultaneously. When the generation of producer gas or another fuel gas rich in carbon monoxide is desired, mixtures of steam and air or air or oxygen alone or suitable mixtures thereof are supplied to the gasification zone in the proper proportions to generate the heat required to raise the burned coke to the temperature necessary for heat balance in the coking zone and to support the desired gasification reaction.

In a more specific modification of this embodiment of my invention just enough air is supplied to the gasification zone to raise the temperature therein to 1600°-1800° F., or higher. Under these conditions the gas leaving the gasification zone contains up to about 30-35% of carbon monoxide and may, after dust separation and desulfurization, be utilized as fuel gas for heating purposes or as fuel for gas turbines or blowing engines.

Independent of the type of fuel gas produced, the gasification zone is preferably so operated that an amount of coke, roughly corresponding to that newly formed in the coking zone, is gasified so that the amount of circulating solids may be maintained at a substantially constant level by merely bleeding off a small amount of ashy or other non-combustible solid constituents which may in turn be used to preheat the oxidizing gas and/or steam required for gasification.

Another embodiment of my invention involves the use of a separate zone for conducting the combustion to supply the heat required for oil-coking and coke-gasification. In accordance with this embodiment of my invention, coke from the oil-coking and/or a fuel gas generating zone is passed, preferably continuously, to a third fluidized solids zone wherein the coke is subjected to combustion with an oxidizing gas, such as air and/or oxygen, at temperatures ranging from 1600° to 2500° F. if desired in the presence of steam or other auxiliary gas which may also aid in the fluidization of the coke. Solid combustion residue and/or other non-combustible solid is returned, preferably continuously, to both the oil-coking and fuel gas

generating zones to supply at least a portion of the heat required therein. If desired, additional heat may be generated within the coking and/or gasification zone by supplying air and/or oxygen directly to said latter zones.

A more specific modification of this latter embodiment of my invention provides for adjusting the amount of oxidizing gas in the combustion zone so as to produce a gas of relatively high carbon dioxide content at temperatures ranging from 1700° to 2500° F. and returning this gas, preferably continuously, together with steam to the gasification zone operated at about 1600°-2400° F. This results in the reduction of carbon dioxide to carbon monoxide by the highly heated coke present in the gasification zone and the conversion of steam to carbon monoxide and hydrogen. The composition of the fuel gas produced in the gasification-reduction zone may be varied by varying the proportions of steam and coke, by charging additional coke or coal or carbureting oil or by similar means. An amount of solid residue approximating the ash content of the residual oil charge may be purged from the system and used for heat exchange purposes, as indicated above. When oxygen alone is used as the oxidizing gas in the combustion zone, the combustion gas may be charged to the reducing-gasification zone directly. When air is used, it may be desirable to concentrate carbon dioxide by scrubbing to eliminate part or all of the nitrogen and to return the concentrated carbon dioxide to the reducing-gasification zone after suitable preheating.

From the foregoing, it will be readily understood that my invention provides a continuous oil-coking process which, in addition to more valuable hydrocarbon coking products, affords full utilization of the carbonaceous matter charged in the form of highly valuable fuel gases while confining the disposal of non-process solids to relatively minor quantities.

Having set forth the general nature and objects, the invention will be best understood from the more detailed description hereinafter, in which reference will be made to the accompanying drawing wherein

Fig. 1 is a semi-diagrammatic view in sectional elevation of an apparatus for carrying out the present process in two separate zones, and

Fig. 2 is a semi-diagrammatic view in sectional elevation of an apparatus for carrying out the present process in three separate zones.

Referring now to Fig. 1, numeral 1 denotes the coking chamber or coker which is in the form of a cylindrical vessel fitted with a conical base 2 separated from the cylindrical section by a distributing grid 4. To start the process, the cylindrical section of coker 1 is filled to about one-third to one-half of its height with a finely-divided solid material supplied by any suitable means, for instance by a screw conveyor 6, as shown in the drawing. The finely-divided solid material should have a particle size of the order of below 50 mesh, or even less than 100 mesh, although even small lumps up to  $\frac{1}{4}$ " or  $\frac{1}{2}$ " size may be used. Coke, preferably oil coke, of the proper size is normally used although any non-combustible solid material, such as sand, ash, catalyst, etc., may take the place of coke in this stage of the process. A fluidizing gas, such as steam, inert gas, water gas, natural gas, flue gases or the like preheated in heater 8 to about

1000°-1200° F. is supplied through line 9 to the conical base 2 of coker 1 and enters the bed of solids in 1 through distributing grid 4 in amounts sufficient to "fluidize" the bed of solids, that is to convert it to a dense, turbulent mass behaving like a boiling liquid and forming a well-defined upper level 5. Simultaneously, the fluidized mass of solids is preheated by the hot gas to the desired coking temperature of 800°-1200° F., or slightly above. Gas volumes of 100 to 1000 cu. ft. per hour and cu. ft. of coker space are normally adequate for this purpose, although these values may vary according to the nature and size of the solids circulated. When the fluidized mass has reached a suitable coking temperature, a heavy hydrocarbon residue, such as reduced crude which may or may not be preheated, is introduced through line 12 into coker 1, preferably at a point above grid 4. The oil is quickly distributed throughout the highly-heated fluidized mass of solids and subject to the coking reaction. It may be desirable to add an oxidizing gas, such as air and/or oxygen, to the fluidizing gas to supply additional heat by partial combustion particularly during the starting-up period.

Volatile coking products, such as gas oil, gasoline and gaseous hydrocarbons together with fluidizing gas are withdrawn overhead from coker 1 and passed through gas-solids separator 13 and line 14 to any conventional system for the recovery of these hydrocarbons (not shown).

Solid fluidized coke is withdrawn downwardly from a point above grid 4 through line 16 to dispersing chamber 18. If desired, the flow of the coke through line 16 may be facilitated by the addition of small amounts of fluidizing gas through lines 17. In dispersing chamber 18 the coke is converted into a suspension of lesser density by the addition of a gas, preferably an oxidizing gas, such as air or oxygen, to which steam may be added and which is supplied through line 19. The suspension formed is passed through line 20 under the pseudo-hydrostatic pressure of the fluidized coke column in line 16 and enters a cylindrical fuel gas generator 22 through a conical base 23 and distributing grid 24 to form above grid 24 a dense, fluidized, turbulent mass similar to that in coker 1 and having a well-defined upper level 25. An oxidizing gas, such as air or oxygen, and/or steam, which during the starting period may be partially or completely replaced by flue gas and preheated in heater 21 to temperatures of the order of 1600°-2500° F., are supplied through line 28, conical base 23 and grid 24 to generator 22 in proportions and amounts, together with gas supplied through line 19, adapted to convert a substantial portion of the coke into a fuel gas, comprising mixtures of carbon monoxide and hydrogen, and to supply sufficient heat by combustion of coke to support the endothermic gasification reaction.

Fuel gas is withdrawn overhead from generator 22 through line 30 and gas-solids separator 32 which may be a centrifugal or electrical type separator and which returns separated solid fines through line 33 to generator 22. Fuel gas substantially free of solids passes through line 34 to reduced crude preheater 36 where it may give off some of its heat to the reduced crude feed supplied by pump 37 through line 38 and passed through line 12 to coker 1. If desired, part or all of the reduced crude feed may by-pass preheater 36 through line 39. The fuel gas leaving pre-

heater 36 is passed through line 40 to storage or further processing (not shown).

Solid gasification residue is withdrawn from a point above grid 24 downwardly through pipe 42. A major portion of the residue is returned about at the temperature of the gasification zone through line 43 to coker 1, preferably at a point above grid 4 and in amounts sufficient to supply the heat required by the coking reaction in coker 1. A considerably smaller portion of solid gasification residue, approximately corresponding to the ash and otherwise introduced non-combustible solids content of the charge, is passed through line 44 to steam preheater 46 which may have a construction similar to that of vessels 1 and 22. Steam or a mixture of steam and oxidizing gas enters preheater 46 through line 47, the conical bottom section 48 and distributing grid 49 to be preheated to the desired temperature by direct heat exchange with the non-combustible gasification residue forming a fluidized mass with a level 50 in preheater 46. Preheated steam or steam-oxidizing gas mixture is passed through lines 51 and 28 to generator 22. Solid residue is withdrawn downwardly from preheater 46 through line 52 and may be passed either through line 53 to disposal means 54 or through line 55 to line 9 to preheat the fluidizing gas for coker 1 by the remaining sensible heat of the non-combustible solid residue.

When the temperature in generator 22 is sufficiently high to make available the heat required in the coker 1 and the steam preheater 46, the process will be self-supporting with respect to heat balance, the total heat required being supplied by the exothermic combustion reaction in generator 22. From this time on, fluidizing gas heater 8 and oxidizing gas heater 21 may be bypassed through lines 10 and 29, respectively. The process may be completely balanced and made fully continuous by so controlling the gasification and combustion reactions in generator 22 that approximately the same amount of coke is converted into gaseous products as is formed in coker 1, fluidized coke being continuously circulated through the system as a heat carrier and oil residue being continuously fed to coker 1.

The amounts of coke returned from generator 22 to coker 1 depend to some extent on the temperature difference between generator 22 and coker 1 and the characteristics of the oil residue to be coked in coker 1. The temperatures in generator 22 will run from 1600° to 2500° F. The proportion of oxidizing gas supplied varies in accordance with the amount of preheat employed, but will generally run about 0.25-0.35 cu. ft. of free oxygen content per cu. ft. of  $\text{CO} + \text{H}_2$  produced in the generator. If the hydrogen content of the gas generated is of no significance, as for instance when producer gas for fuel is desired, the proportion of steam introduced with the oxidizing gas may be only that required for fluidizing or other physical considerations. If higher ratios of hydrogen are required, steam must be added, as for instance in preparing water gas having a  $\text{H}_2:\text{CO}$  ratio of 2:1 for use as feed gas for hydrocarbon synthesis, when as much as 1.5-2.0 cu. ft. (0.07-0.10 pounds) of steam per cu. ft. of  $\text{H}_2 + \text{CO}$  is charged. It will be understood that steam and oxidizing gas, instead of being supplied simultaneously to generator 22, may, if desired, be fed alternately, resulting in a make and blow operation of generator 22. Whenever gases of low nitrogen content, such as hydrocarbon-synthesis gas, are de-

sired oxygen is used as the oxidizing gas. The B. t. u. content of the fuel gas produced may be increased by the addition of a carbureting oil admitted through line 58 to generator 22. The entire system or either one of the reaction zones may be operated at slightly reduced, atmospheric or somewhat elevated pressures, ranging preferably from 25-125 lbs. per sq. in. gauge.

In the embodiment of my invention illustrated in Fig. 2 the heat required in the coking and gasification zones described in connection with Fig. 1 may be generated in a separate combustion zone and the carbon dioxide content of the combustion gases converted to additional amounts of fuel gas. Referring now to Fig. 2, the process is started up in a manner similar to that outlined in connection with Fig. 1. That is to say, coker 201 is charged with a limited amount of finely-divided, if desired non-combustible, solids through screw feeder 206 and a fluidized solids bed is formed in 201 by means of a fluidizing gas preheated in 208 and supplied through line 209 to the conical base 202 below grid 204 in coker 201. Oil residue, such as reduced crude, is fed through line 212 and coked by the heat of the fluidized solids bed. Volatile coking products are taken overhead through separator 213 and line 214 and coke is withdrawn downwardly through line 216 to dispersing chamber 218 where it is dispersed in combustion gases rich in carbon dioxide and steam recovered from the system, as will appear more clearly hereinafter. During the starting period until there is sufficient combustion gas available an auxiliary fluidizing gas from any convenient source pre-heated in heater 221 may be supplied through line 219a to dispersing chamber 218.

The coke dispersion formed in 218 is passed through line 220 to the conical base 223 below distributing grid 224 of gas generator 222 wherein it forms a dense, turbulent, fluidized mass having a level 225. Temperatures within the range of 1600°-2400° F. and relative proportions of carbon dioxide, steam and coke in generator 222 are so controlled as to reduce the carbon dioxide to carbon monoxide and to convert the steam and a substantial portion of the coke into carbon monoxide and hydrogen. Fuel gases are taken overhead through gas-solids separator 232 and line 234 and passed to storage or further processing through reduced crude preheater 236 which may receive the fresh reduced crude feed from pump 237 through line 238 or which may be bypassed by the reduced crude through line 239. The reduced crude feed wholly or partly pre-heated reaches coker 201 through line 212.

A major portion of the hot fluidized solid gasification residue is withdrawn downwardly from generator-reducer 222 at a point above grid 224 and passed to dispersing chamber 241 through line 242. An oxidizing gas, such as air and/or oxygen, which during the starting period may be preheated in heater 227 on line 226, is supplied from gas feed line 241 through preheater 246 where it is in heat exchange with a minor portion of solid gasification residue or otherwise introduced non-combustible solid, as outlined in connection with preheater 46 of Fig. 1, and from there through line 228 to dispersing chamber 241. The coke dispersion which now has a temperature of between 1600° and 2500° F. is passed under the pseudo-hydrostatic pressure of the fluidized solids column in 242, through line 243 into the conical base 260 below grid 261 of the cylindrical combustion chamber or burner 262 wherein it forms

a dense, fluidized mass of solids having an upper level 264.

A minor proportion of fluidized solid gasification residue or otherwise introduced non-combustible solid, roughly corresponding to the non-combustible solids content of the charge, is withdrawn from generator-reducer 222 through line 244 and passed in heat exchange with oxidizing gas through preheater 248, as outlined before. Solid non-combustible residue is removed from the system via line 253 and disposal means 254. The solid may be recycled to the preheater as desired.

In burner 262 the coke is subjected to combustion at temperatures falling within the range of 1700°-2500° F. and under conditions favoring the formation of high proportions of carbon dioxide. For instance, temperatures of 1900° F. at a ratio of 170 cu. ft. of air per pound of carbon content of all fluidized solids entering burner 262 may be advantageously employed.

Hot combustion gases rich in carbon dioxide are withdrawn overhead from burner 262 through gas-solids separator 266 from which separated solids are returned to burner 262 through line 265. The hot combustion gas substantially free of solids passes through line 268 to waste heat boiler 271 in which superheated steam is produced from water supplied through 269; steam is withdrawn through line 270 and mixed with the combustion gases in line 219 leading to dispersing chamber 218 via compressor 272. If desired, inert gases, such as nitrogen, may be removed from combustion gases in a carbon dioxide concentration system 274 arranged in by-pass line 275, and re-heated in heater 276 prior to their admixture with steam in line 219.

A major portion of the mixture of fluidized solid combustion residue and otherwise introduced non-combustible solid is withdrawn at the burner temperature from burner 262 at a point above grid 261 and passed through line 278 to generator-reducer 222, preferably at a point above grid 224 and in amounts sufficient to supply the heat required by the gasification-reduction reaction in chamber 222. A minor portion of the solid fluidized combustion residue is withdrawn from burner 262 in a similar manner through line 280 and passed to coker 201 in amounts sufficient to supply the heat required by the coking reaction.

When the temperature in burner 262 is sufficiently high to make available the heat required in coker 201 and generator-reducer 222 through recirculated hot solid, the process will be self-supporting with respect to heat balance, the total heat required being supplied by the exothermic combustion reaction in burner 262. At the same time the operation of heaters 208 and 227 may be discontinued and the gases by-passed through lines 210 and 228, respectively. The gasification of coke in 222 and the combustion of coke in 262 are preferably so controlled that the amount of coke converted into gas corresponds roughly to that formed in coker 201. Thus, the process may be balanced and made fully continuous by continuously feeding heavy oil residue to coker 201, continuously circulating hot solid composed largely of coke as heat carrier through the system and continuously withdrawing volatile products and small amounts of ashy or other non-combustible solid constituents from the system. In this manner, the carbonaceous constituents of the charging stock are practically completely converted into valuable volatile fuels with only

minor quantities of non-combustible solid residues to be disposed of.

The absolute and relative amounts of solids circulated to and from burner 262 depend within fairly wide limits on the temperature difference between burner 262 and the other conversion zones, the reaction desired in generator-reducer 222 and the characteristics of the original charging stock. In general, operative conditions fall within the approximate limits of 0.5 lb. to 3 lbs., preferably 1 lb., of hot solids recirculated to coker 201 per pound of liquid feed charged to coker 201 and 1 lb. to 4 lbs., preferably 3 lbs., of hot solids recirculated to generator 222 per cu. ft. of CO+H<sub>2</sub> formed in generator 222. Similar considerations apply to the proportions of reacting gases supplied to burner 262 and generator-reducer 222. However, gas ratios of 0.2 cu. ft. to 0.4 cu. ft. of oxygen fed to burner 262 and 0.5 cu. ft. to 1.0 cu. ft. of carbon dioxide plus steam (measured at 60° F. and 1 atm. abs. pressure, whence 2 lbs. of steam=21 cu. ft.) fed to generator-reducer 222 per cu. ft. of CO+H<sub>2</sub> formed will in general be operative. Preferred ratios are 0.25 cu. ft. of oxygen (e. g., in air) and 0.60 cu. ft. of carbon dioxide plus steam.

It is pointed out that this embodiment of my invention permits of many modifications. For example, an oxidizing gas may be fed to coker 201 and/or generator-reducer 222 continuously or periodically to supply additional heat by combustion within said zones or to modify the composition of the volatile products. The fuel gas produced in generator-reducer 222 may be enriched in heating value by injecting a carbureting oil, such as a gas oil, through line 258. Hot solid fluidized gasification residue from line 242 may be returned through line 282 and dispersing chamber 284 to the fluidizing gas line 209 of coker 201 in order to supply additional heat to the fluidizing gas and the coker. On the other hand, part or all of the coke withdrawn from coker 201 through line 216 may be passed through line 286 to a dispersing chamber 288, and picked up by oxidizing gas coming from line 228 through line 290, and then passed as a dispersion through line 292 directly to burner 262. If desired or in case the ash constituents of the reduced crude charged should be insufficient to supply sufficient heat to preheater 246, suitable amounts of extraneous inert solids, such as sand, ash and the like, may be fed to coker 201 and/or burner 262, for instance suspended in the gases supplied to these zones, and circulated through the system with the coke as additional heat carrier. The process may be operated at slightly reduced, atmospheric or slightly elevated pressures, preferably ranging from 25 to 125 lbs. per sq. in. Also, it will be understood that generator 222 may be operated to produce merely carbon monoxide and hydrogen from steam and coke by omitting the carbon dioxide feed from burner 262. Through any or all of these modifications the process become extremely flexible and may be easily adapted to all types of charging stock and volatile fuels desired.

The apparatus of the present process is constructed for operation at relatively low pressure but high temperatures are required especially in the gas generation zones and in the associated pipes. The equipment should be lined with high temperature tile or brick and it is found that there need be little wear if the velocity of the fluidized stream is kept down in the range of 25-75 ft. per second. The operation of the re-

action zones is smooth and proceeds without difficulty. The upward gas velocity should be of the order of 0.5-3 ft. per second where the solid is, say, 50-200 mesh, and progressively higher with larger sizes, say 10-20 ft. per second with lumps  $\frac{1}{4}$ - $\frac{1}{2}$  inch. These velocities are sufficient to prevent the settling of the solid into compact masses and the reactions occur very rapidly when carried out while the solid is in a fluidized condition. Moreover, temperature control is extremely accurate. The minimum velocity of the gas required for maintaining a fluidized condition varies somewhat with the nature and size of the solid particles and the particular fluidizing gas but in general the variation is not wide and the minimum amount is of the order of 0.01-0.10 cu. ft. per lb.; it may consist of gas associated with the solid as withdrawn from a zone of greater gas concentration, without the necessity for adding other fluidizing gas. When fluidizing with such a small amount of gas, a very dense suspension or stream results and the effect of adding additional gas to the fluidized stream is the reduction of the density of the suspension. Advantage is taken of this property of the fluidized stream in order to effect the flow of the material from zone to zone. Thus, in Fig. 1, the stream is caused to flow down the pipe 16 and up the pipe 20 by the addition of gas at the point 18. The density of the fluidized stream in the pipe 16 is much greater than in the pipe 20 and a pressure differential is thus generated, which is equal to the product of the height of the column in pipe 16 multiplied by the density therein, minus the product height of the column 20 multiplied by the density of the stream flowing therein. The equipment should be carefully designed throughout so that the pressure differential is sufficient to overcome the loss due to friction. Small amounts of gas may be added to pipes and chambers at various points so as to maintain the fluidization. This is particularly important where a fluidized stream is flowing downwardly through a pipe wherein the ratio of increase in absolute pressure is of the order of one-tenth or more.

My invention will be further illustrated by the following specific example which is not to be construed as limiting the scope of my invention in any respect whatever.

#### Example

Referring to Fig. 2, a charge consisting of about 100 lbs. of reduced crude is fed in continuous fashion to vessel 201 containing fluidized non-combustible solids at a temperature of approximately 900° F. The oil is coked to produce approximately 45% by weight of gas oil, 16% gasoline and 10% gas. The solid coke is present in the form of a finely-dispersed suspension. During the same time interval, 85 to 100 lbs. of coke or mixtures of coke and non-combustible solids are introduced at a temperature of about 2200° F. Approximately 140 lbs. of solid material withdrawn from the bottom of vessel 201 through standpipe 216 is fluidized by means of air or oxygen-enriched air.

The mixture of air and solid is injected into the combustion chamber 262 in which enough of the combustible in the solid is burned to produce a temperature of 2200° F., approximately 700 cu. ft. of air being required for the purpose of producing the desired temperature level. About 100 lbs. of solid material (combustion residue) are drawn off from combustion chamber

## 11

202 and returned to the coking vessel 201. Approximately 30 lbs. are charged to the gasification vessel 222 in which a substantial portion of the residual carbonaceous material is converted to a gas rich in carbon monoxide when blown with air or oxygen at a temperature of 1810° F. or higher. When operating the gasification chamber 222 with a superficial gas velocity of about 0.8 ft. per second, a producer gas containing 34% CO was manufactured when using air as the 10 oxidizing gas.

Many modifications of my invention will be apparent to those skilled in the art without departing from the spirit of my invention.

I claim:

1. In the method of coking heavy residual hydrocarbon oils wherein subdivided product coke is circulated in a fluidized system comprising a combustion zone and a coking zone and heated substantially above coking temperature while circulating through said system, the improvement which comprises intimately contacting an oil residue of the character of reduced crude at coking temperatures substantially above 800° F. and up to about 1200° F. with a dense fluidized bed of finely divided solid materials substantially free of distillable constituents and comprising non-combustibles to coke said oils, recovering volatile coking products from said coking zone, withdrawing fluidized coke from said coking zone, passing at least a portion of the coke so withdrawn directly to a separate gasification zone, reacting said coke with steam in said gasification zone in the form of a dense fluidized mass of solids at a temperature higher than said coking temperatures to produce a fuel gas, recovering said fuel gas separately from said volatile products, passing ungasified coke from said gasification zone to a separate combustion zone, subjecting said ungasified coke in said combustion zone to combustion in the form of a dense fluidized mass of solids to produce a combustion gas and solid residue heated to a temperature higher than said gasification temperature, withdrawing said combustion gas separately from said fuel gas and said volatile products, controlling said gasification and combustion so as to convert to gas an amount of coke cor-

## 12

responding approximately to the amount of coke formed in said coking zone, passing solids at about the temperature of said combustion from said combustion zone to said gasification zone in amounts sufficient to supply at least a portion of the heat required in said gasification zone, and returning solids heated in said system to a temperature higher than said coking temperature to said coking zone in amounts sufficient to supply at least a portion of the heat required in said coking zone.

2. The method of claim 1 in which at least a portion of said solids returned to said coking zone is withdrawn from said combustion zone.

15 3. The method of claim 1 in which at least a portion of said solids returned to said coking zone is withdrawn from said gasification zone.

4. The method of claim 1 in which carbon dioxide contained in said combustion gases is supplied to said gasification zone and reduced to carbon monoxide by the coke present in said gasification zone.

20 5. The method as claimed in claim 1 in which extraneous solids are added to said fluidized solids passed from zone to zone.

25 6. The method as claimed in claim 1 in which an amount of fluidized non-combustible solids approximately corresponding to the amount of non-combustibles charged to the system is withdrawn from the system.

BRUNO E. ROETHELI.

## REFERENCES CITED

The following references are of record in the 35 file of this patent:

## UNITED STATES PATENTS

| Number       | Name             | Date          |
|--------------|------------------|---------------|
| 1,899,887    | Thiele           | Feb. 28, 1933 |
| 40 1,984,380 | Odell            | Dec. 18, 1934 |
| 2,400,075    | Claussen         | May 14, 1946  |
| 2,436,160    | Blanding         | Feb. 17, 1948 |
| 2,436,938    | Scharmann et al. | Mar. 2, 1948  |
| 2,445,328    | Keith            | July 20, 1948 |

## OTHER REFERENCES

Haslam et al.: "Fuels and Their Combustion," pages 546-547.